

March 22, 1927.

W. O. ALDRICH

1,621,705

MANUFACTURE OF BOLSTER CASES

Filed Jan. 20, 1923

*Fig. 1.*



*Fig. 2.*



*William O. Aldrich*  
INVENTOR  
BY  
*Jeffrey, Kimball & Taylor*  
ATTORNEY

Patented Mar. 22, 1927.

1,621,705

# UNITED STATES PATENT OFFICE.

WILLIAM O. ALDRICH, OF WHITINSVILLE, MASSACHUSETTS, ASSIGNOR TO WHITIN MACHINE WORKS, OF WHITINSVILLE, MASSACHUSETTS, A CORPORATION OF MASSACHUSETTS.

## MANUFACTURE OF BOLSTER CASES.

Application filed January 20, 1923. Serial No. 613,839.

The invention relates to the manufacture of cast iron oil boxes, such as the bolster cases for the spindles of spinning and twisting machinery, and its object is to render 5 such cases proof against leakage of lubricating oil. In the manufacture of spinning and twisting machines, it is found most practical to cast the bolster cases from the same melt as the other heavier, cast iron 10 parts of the machine, the preparation of a special melt or the use of a special metal for these small parts being undesirable on account of the extra expense involved. But when bolster cases are cast of the same metal 15 as the larger castings, a considerable wastage occurs, because many of the cases have to be thrown out because they are not oil-tight. The leakage is found to be due to the relatively coarse grain of the quality of cast 20 iron that is desirable for the larger parts, and its consequent porosity, which permits a slow but highly objectionable escape of lubricating oil to the exterior of the case, where it is likely to soil the yarn. The ob- 25 ject of this invention is to provide an inexpensive means of avoiding such waste while retaining the economy of using the same kind of iron and to this end the invention consists in the impregnation of the surface 30 of such iron castings with a material non-soluble in lubricating oil and capable of stopping the pores of the metal so as to prevent leakage. Several pore-stopping materials are available for this purpose, but the 35 invention particularly and specifically consists in the use of a metallic material and in its impregnation into the cast-iron surface by the process of electro-deposition. The drawing shows, by way of example, in Figure 1 a bolster case of the kind referred to, and in Figure 2 a very much enlarged section 40 of the wall thereof illustrating the surface impregnation by the shade lines.

After being internally bored and externally threaded, the cast iron bolster cases are suspended in a suitable electrolyte bath in the usual manner and the metal, for example nickel, is caused to be deposited thereon. It is sufficient if the deposit is made 45 on either the inside or the outside surface of the case, but it is generally more convenient if it is made on both sides, as shown by Fig. 2. In either case only a slight deposit is necessary, much less than would be required if the bolster case were to be completely nickel-plated. The effect of a slight electrodeposit on the rough, and for the most part porous cast iron, as just described, is to cause the penetration of the metal into the minute granular interstices 55 or pores of the cast surface, and this very slight deposit suffices to stop all the microscopic leak paths through the cast iron wall. No preliminary dressing or grinding of the surface is necessary and it is desirably left 60 rough showing the grain of the molding sand and the marks of the boring or turning tools; nor is any subsequent buffing or other treatment required or desirable after deposit, since the requisite deposit is not heavy 65 enough to take a polish. The deposition need be carried only to the extent of slightly frosting the surface and not to that extent 70 which would cover or conceal the texture of the surface. To carry it to the latter extent would not add to the leak-proof effect 75 and would tend to nullify the advantage and object of the process which, as already stated, are economy of manufacture, but, of course, the extent of the deposit is optional. 80 The present process in its preferred form is thus similar to the common process of electro-plating on cast iron, but differs therefrom, first, in that the cast iron surface is not smoothed or ground in advance of the 85 deposition and, second, in that the process is complete as soon as a change of surface color is observed, which occurs very quickly, as will be understood. The preferred form 90 of the invention thus, in effect, consists of a partial plating on a rough surface.

In actual practice the new process has resulted in the saving of from 10 to 15 per cent of the product, which amount has heretofore been lost on account of oil leakage, 95 besides which the frosted surface gives a pleasing appearance and does not require painting to be commercial, thus increasing the economy, although the cases may be painted, if desired.

I claim:

1. In the art of manufacturing textile machinery, the improvement which consists in casting bolster cases out of the same iron metal from which the frame members of said machinery and other heavier parts are cast, boring and threading the so-cast cases, and then by electro-deposition impregnating the

surface pores of the cases with a permanent metallic frosting and thereby stopping leakage through the pores of the cast iron.

2. The process of manufacturing oil-proof bolster cases, which consists in casting such cases of cast iron, electrodepositing metal into the cast iron surface to an extent only sufficient to produce a frosted appearance on

said surface and thereby stop leakage through the cast iron, and thereafter assembling such cases in a spinning or twisting machine without polishing the surfaces thereof. 10

In testimony whereof, I have signed this specification.

WILLIAM O. ALDRICH.